

June 24, 1930.

F. A. HOWARD

**1,767,455**

550. T. A. HOWARD  
METHOD OF SIMULTANEOUSLY PRODUCING LIGHT HYDROCARBON  
MOTOR FUEL OIL AND CARBURETED WATER GAS  
Filed Nov. 5, 1923

Filed Nov. 5, 1923



## UNITED STATES PATENT OFFICE

FRANK A. HOWARD, OF ELIZABETH, NEW JERSEY, ASSIGNOR TO STANDARD OIL DEVELOPMENT COMPANY, A CORPORATION OF DELAWARE

METHOD OF SIMULTANEOUSLY PRODUCING LIGHT HYDROCARBON MOTOR FUEL OIL AND CARBURETED WATER GAS

Application filed November 5, 1923. Serial No. 673,015.

This invention is a method of jointly manufacturing carbureted water gas and volatile hydrocarbon motor fuels and will be fully understood from the following 5 specification.

It is well known that relatively heavy hydrocarbon oils, such as petroleum distillates having a boiling point range from 450° F. to 800° F., are well adapted for

10 gas manufacture by cracking. This process is usually carried out in connection with the manufacture of blue gas or water gas, in which case the oil is vaporized and cracked in one part of a combination apparatus, another part of which is employed for furnishing the heat for the entire operation and for making the water gas by alternately serving as a gas producer and as a water gas generator. It is characteristic of 15 this process that the cracking of the oil is carried on in an atmosphere of blue water gas, that is, an atmosphere of which hydrogen represents about 50%, neglecting undecomposed steam.

20 In accordance with this invention, the peculiar conditions which obtain under these circumstances are controlled and utilized to produce simultaneously, and efficiently and in maximum quantity both gas of the 25 desired calorific value or B. t. u. rating and low-boiling oils (boiling, say, below 400° F.).

In the accompanying drawing a combination water gas generator and oil cracking 30 apparatus suitable for carrying out the invention is shown in vertical section.

In the drawing the numeral 5 designates a water gas generator, which is charged with fuel (coal, coke, etc.) through charging 35 door 6, the fuel bed being indicated by numeral 7. Air for blasting is supplied through valved pipe 8. Steam may be supplied below the fuel bed through valved 40 steam pipe 9 or above it through tuyères 10 supplied from valve-controlled header 11. Valved gas outlets 12 and 13 from the generator 5 are provided above and below the fuel bed respectively, leading into the inlet 45 pipe 14 to the carbureter 15. A valved pipe 50 16 for air opens into the top of the carbu-

reter. The carbureter is provided internally with checkerwork 17. At its top is a spray pipe 18, which may be fed with oil through valved pipe 19 or with steam through valved pipe 20.

From the carbureter 15 an outlet or throat 21 leads into the superheater 22. A valved pipe 23 for supplying air may be tapped into the bottom of superheater 22. The superheater 22 is provided internally 55 with a checkerwork 24. Its top is closed by valve 25, directly below stack 26. An outlet pipe 27 provided with a valve 28 leads into the top of the condenser or wash box 29, which is provided with a spray pipe 30 through which water may be introduced. Near its base the condenser 29 is provided with a liquid overflow pipe 31 which leads 60 into a separator 32. A valved gas pipe 33 makes communication between the wash box 29 and separator 32 above the liquid levels 65 therein. The separator 32 is provided with a partition 34 which is located at some distance from the inlets of pipes 31 and 33 and extends downwardly from the top of 70 the separator to below the liquid level therein and terminates somewhat above the bottom of the separator. A gas withdrawal pipe 36 and an oil overflow pipe 37 are located on the same side of the partition 34 75 as the inlets of pipes 31 and 33. On the other side of said partition the separator 32 is provided with a water overflow pipe 35. The oil overflow pipe 37 terminates in 80 an open end located above the connection of pipe 35 so that oil passes off by pipe 37 and water by pipe 35. The gas pipe 36 leads to a suitable gas holder (not shown).

The operation of this apparatus is as follows: The generator 5 is blasted with air 85 through pipe 8, the depth of the fuel bed being so great that the combustion gases are more or less rich in carbon monoxide. These gases pass on through the checkered spaces of the carbureter 15 and superheater 90 22. Air may be admitted either into the top of carbureter 15 through pipe 16 or into the bottom of superheater 22 through pipe 23 or both as required to produce the requisite 95 amount of combustion to raise the tempera- 100

ture of the checkerwork 17 and 24 to the desired points. By varying the air blast to the fuel bed of the generator to regulate the CO content of the gas produced, and by control of auxiliary air, the temperatures 5 may be regulated through a very wide range. During this time the stack valve 25 is open. When the fuel bed, carbureter and superheater have reached the operating 10 temperatures, the air blast is shut off and valve 25 is closed. Steam is admitted either to the top or bottom of the generator, passing up or down as the case may be, to be decomposed with the liberation of hydrogen 15 and the simultaneous production of carbon monoxide and forming blue water gas.

The mixture of carbon monoxide, hydrogen and undecomposed steam passes from the generator 5 to the top of the carbureter 15, into which the heavy hydrocarbon oil 20 is sprayed through pipe 18. The oil is vaporized almost instantaneously and the vapors carried by the high velocity current 25 of mixed carbon monoxide and hydrogen pass through the heated checkerwork of the carbureter and superheater.

I have discovered that by a proper control 30 of the temperature of the carbureter and superheater, and a proper correlation of these temperatures to the capacity or volume 35 of the system and the rate of flow of the gases and vapors through it (these two last named conditions governing the time element 40 of the cracking), the character and extent of the thermal decomposition of the oil 45 may be controlled to produce a substantial yield of light hydrocarbons suitable for motor fuel. At the same time, the process 50 of water gas manufacture and carburetion for which the apparatus is primarily designed, may be carried on without loss of efficiency or capacity, the production of motor fuel being made an incident of the regular operation of the carbureted water gas plant. In this way, the conversion of a certain proportion of the oil treated into permanent gas—which is an undesirable incident and an economic loss in an ordinary cracking process for producing motor fuel 55 from heavy hydrocarbon oil—becomes an economically desirable feature.

In carrying out the present invention, the successive operations of blowing, simultaneous gas making and oil feeding, and purging 60 are carried out along the general lines of established water gas manufacturing practice, the periods during which the successive operations of each cycle are conducted being determined, however, by the temperature 65 conditions which it is desired shall prevail in the carbureter and superheater. In carrying out the process, the controlling temperature conditions are preferably selected 70 as those prevailing in the throat 21 and the superheater outlet 27, as temperatures taken

at these points are not greatly affected by radiation from more or less incandescent portions of the apparatus, as is the case with temperature readings taken within the carbureter and superheater. With suitable compensating factors taken into consideration, such internal temperatures may be employed 75 however for control instead of the throat and outlet temperatures, if desired.

In carrying out the operation, the temperature at the throat 21 between the carbureter and the superheater is maintained at 75 from 1200 to 1300° F. and preferably from 1250 to 1290° F. These temperatures are average temperatures, and the variation 80 from maximum to minimum so averaged may be from 150 to 200° F. The temperatures of the gases leaving through the outlet 27 from the superheater are maintained at an average of from 1050 to 1200° F., and 85 preferably between 1100 and 1150° F. The variations of temperature in the outlet so averaged may be from 50 to 75° F. from maximum to minimum.

In running the apparatus, the period of 90 air blasting the fuel bed varies from three to four minutes, the precise time being determined by the temperature in the throat 21 and outlet 27. As soon as the desired temperatures are reached at these points steam 95 is introduced into the generator and oil is simultaneously fed into the carburetor for a period of, for example, two minutes at a suitable rate, which, in the case of a gas set of the size known as an eight foot six 100 inch set, was found to be from 20 to 25 gallons per minute. On larger or smaller sets, the rate of feed of oil may be correspondingly varied. After the period of oil feeding, steam pressure is increased and the apparatus is purged in the usual manner, at 105 the end of which time the cycle is repeated.

Under the conditions described, gas of a calorific value of 580 to 670 B. t. u. per cubic foot is manufactured at a rate of from about 90 to 100% of the rated capacity of the set, and at the same time light oils (boiling below 400° F.) are produced to the extent of 110 15 to 20% of the total oil fed into the set.

The following specific example illustrates 115 more fully the present process, the gas set employed in the tests referred to being known as an 8 ft. 6 in. gas set. The generator was 9 ft. outside diam., 7 ft. inside diam., and 15 ft. high. The carburetor was 8 ft. 120 outside diam., 6 ft. inside diam., and 17 ft. high. The superheater was 8 ft. outside diam., 6 ft. inside diam., and 22 ft. high. The wash-box was 6 ft. diam., by 4 ft. high.

The results obtained in a representative 125 test on the above gas set using a regular, commercial gas oil of 39° Bé., with an initial boiling point of 394° F. and 90% off at 675° F., were as follows:

Duration of test, 3 hr. 43 min.; average 130

length of complete cycle, 7.4 min.; oil per cycle (gallons), 40.6; oil per min. (gallons), 20.3; total oil used (gallons), 1220; percent of total oil recovered as oil, 27.8; percent of oil recovered as oil boiling below 400° F., 18.0; total gas made, cu. ft., 225,900; percent of rated capacity of set, 94; B. t. u. of gas, per cubic foot, 665; average throat temperature, °F., 1276; average outlet temperature, °F., 1129; average steam pressure, down run, lbs. per square inch, 10; average steam pressure, up run, lbs. per square inch, 20.

The light oil is suitable for use as a motor fuel and at least one-half of it consists of paraffin hydrocarbons. It is recovered by partial distillation of the "tar" which condenses in the wash box, scrubber, or condenser with which the water gas set is equipped, and by scrubbing the gas with a suitable absorbing agent in the regular manner heretofore used for recovery of benzol, toluol, etc., from carbureted water gas.

In operating at the rate specified, that is, at 90 to 100% of the rated capacity of the set, 970 to 1080 cubic feet of carbureted water gas per minute are produced. Since the volume (including checker work) of the cracking space, that is, the combined volume of carburetor and the superheater, is about 1102 cubic feet, the gas production is between 880 and 980 cubic feet of carbureted water gas per minute per 1000 cubic feet of checker work packed cracking space.

The oil rate is about 5.4 gallons per 1000 cubic feet of gas produced, that is 15 to 20% greater than the rate normally required for enriching the water gas to the standard B. t. u. rating for illuminating gas. The rate normally required to so enrich the water gas is equivalent to 4.9 gallons per minute per 1000 cubic feet of checker-work packed cracking space.

It will be noted from the foregoing example that there was used 5.4 gallons of oil per 1000 cubic feet of gas produced, and that this gas was of 665 B. t. u. rating. According to ordinary gas practice the production of a gas of this heat value would require approximately 4.5 gallons of oil per 1000 cubic feet, the calorific value of the "blue gas" or water gas being about 300 B. t. u. I therefore employ, according to my process a substantially larger amount of oil than in ordinary practice (20% or more in excess) but so modify the condition of operations that this excess of oil is very largely recovered as a low boiling distillate suitable for motor fuel.

I claim:

1. The method of producing light hydrocarbon motor fuel oil from heavier hydrocarbon oil while simultaneously manufacturing carbureted water gas of predetermined B. t. u. rating; which comprises blasting a

body of incandescent carbonaceous material with steam, thereby producing water gas, passing the water gas over hot refractory material and injecting the heavy hydrocarbon oil thereinto, the temperature of said refractory material being such that the gases and vapors leave it at from 1200° to 1300° F., whereby the gases are carbureted, the proportion of heavy hydrocarbon oil injected being controlled relative to the desired calorific value of the gas in amount corresponding to about 5.4 gallons per thousand cubic feet of gas of 665 B. t. u. rating, passing the resulting gases and vapors over additional refractory material heated to such a temperature that the gases and vapors leave it at a temperature between 1100° and 1200° F., and subsequently condensing and separating from said gases and vapors the condensable low boiling point oil.

2. The method of producing a light hydrocarbon motor fuel oil from heavier hydrocarbon oil and simultaneously manufacturing carbureted water gas of predetermined calorific value; which comprises blasting a body of incandescent carbonaceous material with steam, thereby producing water gas, passing the water gas over hot refractory material and injecting such heavier hydrocarbon oil thereinto, the temperature of said refractory material being such that the mixed gases and vapors leave it at from 1250° to 1290° F., passing the resulting gases and vapors over additional hot refractory material at a temperature such that the gases and vapors leave it at a temperature of 1100° to 1150° F., controlling the proportion of said heavy hydrocarbon oil injected into said gas so that not over about 80% thereof is converted into fixed gas and oil of boiling point above 400° F. while securing finished gas of the desired calorific value, and separating and collecting from the gases and vapors the condensable oils having boiling points below 400° F.

FRANK A. HOWARD.

115

120

125

130